

## UNITED STATES PATENT OFFICE

FRIEDRICH W. WEBER, OF HACKENSACK, NEW JERSEY, ASSIGNOR TO MAYWOOD CHEMICAL WORKS, OF MAYWOOD, NEW JERSEY, A CORPORATION OF NEW JERSEY

## PROCESS FOR WEIGHTING TEXTILE FIBERS AND PRODUCT OBTAINED THEREBY

No Drawing.

Application filed February 3, 1930. Serial No. 425,707.

My present invention relates to improvements in the art of treating fibers and particularly to the art of weighting silk and rayon, the object of the invention being to provide a process whereby both silk and rayon are quickly weighted with less labor and less danger to the operator, and whereby the metal oxides precipitated thereon are so intimately introduced into the fibers so as to give them an excellent whiteness and luster.

The demand of the public to have garments of silk improved in luster and the necessity of weighting rayon to improve the wearing of the light, loosely hanging rayon garments, make it desirable to provide a process which, without affecting the strength of the fiber, will improve the luster and weight of other materials and provide these advantages at a relatively low price.

All processes introduced for this purpose were accompanied by a considerable number of difficulties inasmuch as they were almost exclusively based on the application of tin tetrachloride and its conversion into tin phosphate on the fiber. These difficulties were caused by the corrosive action of the tin tetrachloride solution and were most unpleasantly felt during its mechanical handling, but most important were the complications caused by its chemical properties displayed by the solution in the weighting process proper.

The greatest difficulty in the weighting of the silk is caused by acid and it is natural that up to now only the solutions of practically neutral or only weakly acid salts, as for instance of tin tetrachloride,  $\text{SnCl}_4$ , were found suitable for this purpose. Much hydrochloric acid is split off during the operation with tin tetrachloride and therefore the solutions of this salt, even if always used with certain precautions, became less and less effective the longer they were used, on account of their enrichment with ammonium chloride.

This addition of ammonia became practically indispensable to establish the necessary basicity of the tin solution; but the ammonia applied for this purpose forms ammonium chloride and becomes in the long run a disturbing element and soon the weighting bath does not work properly any more and must be replaced.

In view of the fact that also the efforts of the prior art of weighting silk by means of the insoluble compounds of the rare earth metals have not survived the experimental stage (see Heermann, Faerberei & Textilchemische Untersuchungen, publ. by Julius Springer, Berlin, 1923, p. 202) and as it is stated by Hottenroth, Artificial Silk, publ. by Pitman & Sons, London, 1928, on page 369, that

"It is impossible to weight artificial silk in the manner adopted for natural silk, in which the weighting often amounts to several hundred per cent of the fiber. In so far as proposals for this purpose exist, they are confined to weighting up to 3 to 5 per cent or rarely up to 6 to 10 per cent."

the process of the present application is of all the greater importance because it furnishes not only silk and rayon products of absolute whiteness, but particularly furnishes rayon products showing the same increase in weight as natural silk.

With this situation confronting the silk weighting industry the problem solved by the present invention was to find a de-acidifying agent which could not only be used to de-acidify the metal salts of the weighting bath, but which desirably at the same time also would act as a means for weighting the silk.

Many efforts have been made to obviate the harmful effects of the tin solution; among other suggestions one was added organic additions to the tin solution to bring about a better splitting off of the tin oxy-

hydrate, but it was without avail. Moreover, the old processes always required considerable washing to obtain a satisfactory hydrolytic splitting off of the tin as hydrate, whereby great losses of tin were entailed.

It, therefore, represented a very beneficial contribution to the art when I actually discovered the circumstances under which it was possible to prevent right from the beginning the quick increase in the acid content of the bath by the addition of a substance of such properties to simultaneously obtain a silk considerably increased in weight.

15 The following points had to be considered in my efforts to improve the process:

1. The application of a weighting bath which is inclined to more quickly split off the tin oxy-hydrate without, however, liberating 20 a considerable quantity of free acid and by preventing the formation of this acid for also saving a longer washing of the silk.

2. By the application of a de-acidifying agent of high atomic weight and of a sufficiently low price, but having at the same time an affinity to the silk at least as great as the tin so it could not be considered as a disturbing element.

3. Finally the bath had to be such that its 25 composition and its specific gravity would not change materially so that it could be used for a long time.

Such a de-acidifying agent I found in the carbonates of the rare earths, which, when 35 added to tin tetrachloride split off the chlorine from the same without otherwise causing a disturbance of the solution, and which allow to work therefore right from the beginning with a solution of considerably reduced 40 acidity. My new invention also offers the advantage of applying a substance which under certain circumstances displays or can be caused to display an affinity to the silk fiber and therefore is also capable of being 45 precipitated thereon.

I found that for instance a moderately 50 concentrated tin tetrachloride solution may be de-acidified with carbonates of the rare earth metals without turning smoky, i. e. a considerable amount of mixed carbonates, or even the carbonate of one only, of the rare earth metals, for instance such as lanthanum, didymium, thorium, etc., may be dissolved 55 according to the following equations:



60 in the tin tetrachloride, intended to be applied for weighting, by copiously generating carbon dioxide gas. The purposes intended to be attained by the application of 65 these products and the phenomena accom-

panying the same will be explained below by way of example.

#### Example 1

If for instance 75 grams of thorium 70 carbonate are slowly added to 750 grams of a 50 Bé. tin tetra-chloride solution, heated up to 75° C., they will be quickly dissolved entirely and the solution obtained will show only a faint smokiness which is due to small 75 traces of impurities of the applied thorium carbonate or to those of tin tetrachloride and which can be removed either by filtration or decantation.

The solution thus obtained is immediate- 80 ly ready for application and has only to be adjusted to 36° Bé. to have the proper concentration. The silk is allowed to soak in this tin-thorium oxychloride solution for some time, for instance 1-1½ hours; it is then 85 taken out, the surplus of the solution is thoroughly squeezed out of the silk and the same is then washed with relatively little water. The washed silk is then introduced into a di-sodium phosphate bath having a temperature of approximately 70° C. The silk is allowed to hang therein also for 1½ hours, taken out, washed and dried. This procedure may be repeated once or twice, or as often as desired. The increase in the weight 90 of the silk obtained in its first passage through the bath is considerably greater than with any other solution known in the art of silk weighting up to now.

From former experiences one would logically suppose that such a solution will turn smoky when allowed to stand, or by the repeated passage of the silk through this solution would lose considerably in its concentration, or would otherwise be considerably 105 disturbed in its composition, but this is in no wise the case.

Such permanently clear solutions require, however, that the water be free of certain salts which eventually may precipitate, for 110 instance calcium and iron salts. As the water supply in the silk dyeing plants often does not meet this condition, I may operate the process as described in the following:

#### Example 2

I introduce 750 gr.  $\text{SnCl}_4$  solution, 50° Bé., into a vessel and heat it approximately up to 75° C., whereupon I add 50 gr. of the carbonates of lanthanum and didymium while the solution is agitated. The mixture is heated for some minutes after all the carbonate has dissolved, whereupon water is added to make up 1 liter and the solution is then allowed to cool. Gradually a more or less brown precipitate segregates which is filtered off whereby an absolutely clear solution is obtained, to which I add a certain amount of an organic acid which forms a soluble calcium and iron salt; such acids are 125 130

for instance, formic acid, acetic acid, and similar acids low priced enough and fulfilling the above stated requirements concerning the solubility of its calcium and iron salt. I add 5 for instance to the above quantity of solution 10 gr. of a 98% formic acid or a corresponding amount of any of the other acids. After this last addition the solution shows 31° Bé. and is ready for use.

10 The solutions obtained by the directions of aforesaid examples are particularly suitable for weighting both natural and artificial silk, regardless whether the latter were products of the viscose, the cuprammonium-cellulose, 15 the cellulose acetate or other process, which products I simply embrace henceforth in the general term "rayon".

The above given examples are, moreover, typical only of the variations which I may 20 practise in my new process. It is evident that its simplicity will allow even the operation by a working man, having no chemical training, after a short instruction.

As I already stated above the tin tetrachloride solution, de-acidified by the carbonates of the rare earth metals, would stay clear even without the addition of the acid, but the presence of the same has the considerable advantage, in case of the presence of Ca, or 30 Fe compounds, to prevent their precipitation upon the silk which would render the silk unsightly and thus cause the loss of the silk because these defects can never be remedied.

The new process offers therefore the best 35 possibility of weighting silk with a relatively highly concentrated solution without appreciable losses of tin and with a highly desirable luster.

The tendency of the solution, thus obtained, 40 to precipitate upon silk is much stronger than that of any other solution heretofore applied for the same purpose. This appears due to the fact that the solution after its treatment with the rare earth metals contains the same 45 original amount of acid, but that of this acid a part only is still combined with the tin, while a considerable balance of acid has combined with the rare earth metals, the result being that the solution of the tin and of the 50 rare earth metals shows a very much weakened acid reaction. When the de-acidified solution enters the capillary spaces of the fiber it is hydrolyzed; the solution in said spaces thereby turns rapidly more basic and also 55 easily precipitates the hydrate of stannic acid. A fiber already charged with tin oxy-hydrates shows great affinity for a deposit of the oxy-hydrates of the rare earth metals.

In this process the fortunate result occurs 60 that simultaneously a precipitation of tin oxy-hydrate and of those of the rare earth metals takes place in one treatment, or operation, in the same bath without any disturbance of its quantitative composition, i. e. in 65 the proportion of its ingredients. By this

fortunate combination the present invention offers a distinct advantage over the prior art.

The advantage of my new process over the old tin-tetrachloride process is self evident to one skilled in the art. He finds that without 70 any addition whatever he can obtain for three times in succession, each time with a new skein, the same amount of increase in the weight of the fiber which would be entirely impossible in the  $\text{SnCl}_4$  baths of the prior 75 art on account of its getting continuously more acid. This and similar advantages will soon be apparent to the silk dyer, and particularly that the application of solutions of 80 relatively low acidity harbors less danger to the durability of the fiber.

Also the possibility of using highly concentrated solutions right from the beginning and the great stability of the composition, resulting in a constant clearness, of these 85 highly basic solutions will be appreciated, as well as an immediate increase in weight of the fiber in the double proportion of that obtainable with the old tin tetrachloride process.

Further advantages, which should not be underestimated, reside in the reduction of the great quantities of washing water to complete the splitting of the tin and rare earth metal salts by hydrolysis in the silk and rayon fiber, this quantity of water having been reduced to an indispensable minimum. I have also found that the solution of the di-sodium phosphate acts much quicker on the fibers, treated as described, that therefore this phosphate solution is also better utilized, that the 90 completely weighted product appears to be more voluminous particularly if thorium is applied, and that the produced silk and rayon is always whiter and of greater durability 95 because the conditions for the formation of metastannic acid are removed.

Another advantage, which must be particularly emphasized, is the constant clearness of the solution and that thereby the obtained product is whiter and more lustrous, 110 which is not the case if for instance thorium is applied under other conditions, or if silk is treated only with tin phosphate.

My new process described above is also applicable to other metal solutions used as 115 mordants in the treatment of fibers for dyeing purposes and solutions of iron chloride,  $\text{FeCl}_3$ , and similarly acting salts of the aforesaid and other metals may be treated according to the principle of my new process for 120 various purposes of treating textile fibers, i. e., in place of tin with, for instance, the correspondingly deacidified solutions of iron, aluminum, etc. salts.

The new process brings relief from the 125 various, sorely felt hardships of the tin-tetrachloride bath because the corrosive effect of the same was almost equally as destructive to the containers, tanks, etc. which had to be used in the weighting process, as it was de- 130

structive to the hands and body of the operator. All these hardships are at least reduced to a tolerable degree, if not entirely avoided by my new process.

Moreover, the whole process is more simple, a few steps only being required to obtain a better effect than with tin tetrachloride alone. The simplicity of the whole process speaks for itself and the operation and control of the process can be done by any plain laborer after being once instructed, for a little more of added carbonates of the rare earth metals is far less disturbing than the increase in acid of the tin tetrachloride bath.

This simplicity avoids the close observation which had to be given to each separate tin tetrachloride bath and the many analytical tests to follow up the exhaustion of these baths and the effect of the addition of ammonia on the same.

It is one of the desirable features of my invention that the de-acidification of the tin tetrachloride solution and similar salt solution is effected with a material which in itself is capable of adding weight to both natural and artificial silk; for instance if I apply the carbonate of thorium, which has the high atomic weight of 232, the weighting is effected very quickly and with a considerable saving of material and wages.

The present invention is, moreover, not only of economical importance to the dyer, but is of considerable importance to the manufacturer of chemical products from monazite sand which contains relatively much thorium, which up to now was used in great quantities in the manufacture of gas mantles for incandescent gas light, but with the ever increasing use of electricity for lighting purposes, lost its market.

To obtain the other rare earth metals and their compounds, the manufacturers always have to separate the thorium from the monazite sand and for the present state of the lighting industry the stocks of thorium compounds were ever increasing and swallowing more capital, so that also in this field my new invention brings relief.

Whenever I speak of an alkali metal salt for acting on the basic tin and on the basic rare earth metal salt, I also mean to include the corresponding ammonium salt in the term "alkali metal salt".

What I claim is:

1. The process of weighting textile fibers, said process consisting in acting upon a weighting metal salt solution with the compound of a rare earth metal capable of combining with the acid component of aforesaid metal salt, thereby obtaining a practically clear solution of the reaction products, passing the fiber through the solution of the reaction products, washing the fiber thus treated with water, and then passing the fiber through the solution of a salt capable

of forming an insoluble salt with each of the metals introduced into the fiber.

2. The process of weighting textile fibers, said process consisting in acting upon a weighting metal salt solution with the carbonate of a rare earth metal thereby obtaining a practically clear solution of the reaction products, passing the fiber through the solution of the reaction products, washing the fiber thus treated, and then passing the fiber through the solution of a salt forming an insoluble salt with each of the metals introduced into the fiber.

3. The process of weighting textile fibers, comprising acting upon a weighting metal salt solution with the compound of a rare earth metal capable of combining with the acid component of aforesaid metal salt thereby obtaining a practically clear solution of the reaction products, and subjecting the fiber to said clear solution.

4. The process of weighting textile fibers, comprising acting upon a weighting metal salt solution with the carbonate of a rare earth metal obtaining thereby a practically clear solution of the reaction products, and subjecting the fiber to said clear solution.

5. The process of weighting both natural and artificial silk, said process consisting in acting upon a tin tetrachloride solution with the compound of a rare earth metal capable of combining with the acid component of aforesaid tin tetrachloride solution and thereby obtaining a practically clear solution of the reaction products, passing the silk through the solution of the reaction products, washing the silk thus treated with water, and then passing the silk through the solution of a salt capable of forming an insoluble salt with the tin and the rare earth metal introduced into the fiber.

6. The process of weighting both natural and artificial silk, said process consisting in acting upon a tin tetrachloride solution with the compound of a rare earth metal capable of combining with the acid component of aforesaid tin tetrachloride solution and thereby obtaining a practically clear solution of the reaction products, passing the silk through the solution of di-sodium phosphate.

7. The process of weighting both natural and artificial silk, said process consisting in acting upon a tin tetrachloride solution with the carbonate of a rare earth metal thereby obtaining a practically clear solution of the reaction products, passing the silk through a solution of the reaction products, washing the silk thus treated with water, and then passing the silk through the solution of a salt capable of forming an insoluble salt with the tin and the rare earth metal introduced into the fiber.

8. The process of weighting both natural and artificial silk, said process consisting in

acting upon a tin tetrachloride solution with the carbonate of a rare earth metal thereby obtaining a practically clear solution of the reaction products, passing the silk through the solution of the reaction products, washing the silk thus treated with water, and then passing the silk through a solution of disodium phosphate.

9. The process of weighting both natural and artificial silk, said process consisting in acting upon the solution of a metal salt, suitable as a weighting material for silk, with a thorium compound, capable of combining with the acid component of said metal salt, thereby obtaining a practically clear solution of the reaction products, passing the silk through this solution of the reaction products, washing the silk thus treated with water, and then passing the silk through a solution forming an insoluble salt with aforesaid metal and thorium.

10. The process of weighting both natural and artificial silk, said process consisting in acting upon the solution of a metal salt, suitable as a weighting material for silk, with thorium carbonate thereby obtaining a practically clear solution of the reaction products, passing the silk through this solution of the reaction products, washing the silk thus treated with water, and then passing the silk through a solution forming an insoluble salt with aforesaid metal and thorium.

11. The process of weighting both natural and artificial silk, said process consisting in acting upon a solution of tin tetrachloride with thorium carbonate, thereby obtaining a practically clear solution of the reaction products, passing the silk through this solution of the reaction products, washing the silk thus treated with water, and then passing the silk through a solution forming an insoluble salt with aforesaid metal and thorium.

12. The process of weighting both natural and artificial silk comprising deacidifying a metal salt solution, having weighting properties, by a carbonate of a rare earth metal, thereby obtaining a clear solution of the reaction products, and subjecting the silk to said clear solution.

13. The process of weighting both natural and artificial silk comprising deacidifying a metal salt solution, having weighting properties by thorium carbonate, thereby obtaining a clear solution of the reaction products and subjecting the silk to said clear solution.

14. The process of weighting both natural and artificial silk comprising deacidifying tin-tetrachloride solution with a basic compound of thorium, thereby obtaining a practically clear solution of the reaction products, and subjecting the silk to said clear solution.

15. The process of weighting both natural and artificial silk comprising deacidifying tin tetrachloride solution with thorium carbonate, thereby obtaining a clear solution of

the reaction products, and subjecting the silk to the said clear solution.

16. The method of weighting both natural and artificial silk comprising acting on the silk with a solution of basic metal chlorides, one of the same being a basic tin chloride salt. 70

17. The method of weighting both natural and artificial silk comprising acting on the silk with a solution of tin tetrachloride deprived of its deleterious effect by the action of a thorium carbonate. 75

18. As a base for the weighting of both natural and artificial silk, an aqueous solution of a basic tin chloride and of a basic rare earth metal chloride. 80

19. As a base for the weighting of both natural and artificial silk, an aqueous solution of a basic tin chloride and of a basic thorium chloride. 85

20. The process of weighting textile fibers, said process consisting in acting upon a weighting metal salt solution with a weighting metal compound capable of combining with part of the acid component of aforesaid metal salt, adding to the reaction product an organic acid capable of forming soluble salts with all metals present in the reaction mixture, passing the fiber through the solution of the reaction products, then passing the fiber thus treated through the solution of a substance capable of forming an insoluble salt with each of the metals introduced into the fiber. 90

21. The process of weighting textile fibers, said process consisting in acting upon a weighting metal salt solution with a compound of a rare earth metal capable of combining with the acid component of aforesaid metal salt, adding to the reaction product an organic acid capable of forming soluble salts with all metals present in the reaction mixture, passing the fiber through the solution of the reaction products, then passing the fiber thus treated through the solution of a substance capable of forming an insoluble salt with each of the metals introduced into the fiber. 100

22. The process of weighting both natural and artificial silk fibers, said process consisting in acting upon a tin-tetrachloride solution with a compound of a rare earth metal capable of combining with the chlorine of the tin tetrachloride and thereby dissolving in said solution, adding to the reaction product an organic acid forming a soluble salt with aforesaid metals and with calcium and iron present in the water applied for the solution, passing the silk through the solution of the mixture, and then passing the silk through a solution capable of forming an insoluble salt with the tin and the rare earth metal introduced into the silk. 110

23. The process of weighting both natural and artificial silk fibers, said process consisting in acting upon a tin-tetrachloride so- 120

125

lution with a mixture of the carbonates of lanthanum and didymium, adding formic acid to the reaction product, passing the silk through the solution of the mixture, and then 5 passing the silk through a solution capable of forming an insoluble salt with the tin, lanthanum and didymium.

24. In the process as described by claim 22, the step of adding formic acid to the solution 10 of tin tetrachloride de-acidified by rare earth metals.

In witness whereof, I have hereunto set my hand.

FRIEDRICH W. WEBER.

15

20

25

30

35

40

45

50

55

60

65